



US005681405A

## United States Patent [19]

Newton et al.

[11] Patent Number: 5,681,405

[45] Date of Patent: Oct. 28, 1997

## [54] METHOD FOR MAKING AN IMPROVED ALUMINUM ALLOY SHEET PRODUCT

[75] Inventors: William Newton; David A. Tomes, both of San Antonio, Tex.

[73] Assignee: Golden Aluminum Company, Golden, Colo.

[21] Appl. No.: 401,418

[22] Filed: Mar. 9, 1995

[51] Int. Cl.<sup>6</sup> C22F 1/04

[52] U.S. Cl. 148/551; 148/552; 148/692; 148/439; 420/533; 420/534

[58] Field of Search 148/551, 552, 148/688, 692, 696, 439; 420/533, 534, 537, 538, 542, 546, 547

## [56] References Cited

## U.S. PATENT DOCUMENTS

- |           |         |                 |         |
|-----------|---------|-----------------|---------|
| 4,111,721 | 9/1978  | Hitchler et al. | 148/696 |
| 4,235,646 | 11/1980 | Neufeld et al.  | 148/551 |
| 4,238,248 | 12/1980 | Gyöngyös et al. | 148/551 |
| 4,517,034 | 5/1985  | Merchant et al. | 148/439 |

|           |         |                  |         |
|-----------|---------|------------------|---------|
| 4,526,625 | 7/1985  | Merchant et al.  | 148/439 |
| 4,929,285 | 5/1990  | Zaidi            | 148/692 |
| 4,976,790 | 12/1990 | McAuliffe et al. | 148/551 |
| 5,192,378 | 3/1993  | Doherty et al.   | 148/691 |

## FOREIGN PATENT DOCUMENTS

93304426.5 7/1993 European Pat. Off.

## OTHER PUBLICATIONS

Don McAuliffe, "Production of Continuous Cast Can Body Stock", Paper presented at AIME Meeting, Feb. 27, 1989, 7 pages.

Primary Examiner—George Wyszomierski  
Attorney, Agent, or Firm—Sheridan Ross P.C.

## [57] ABSTRACT

An aluminum alloy sheet and a method for producing an aluminum alloy sheet. The aluminum alloy sheet is useful for forming into drawn and ironed container bodies. The sheet preferably has an after-bake yield strength of at least about 37 ksi and an elongation of at least about 2 percent. Preferably the sheet also has earing of less than about 2 percent.

38 Claims, 1 Drawing Sheet



FIG. 1



## METHOD FOR MAKING AN IMPROVED ALUMINUM ALLOY SHEET PRODUCT

### FIELD OF THE INVENTION

The present invention relates generally to aluminum alloy sheet and methods for making aluminum alloy sheet. Specifically, the present invention relates to aluminum alloy sheet and methods for making aluminum alloy sheet wherein the sheet is particularly useful for forming into drawn and ironed container bodies.

### BACKGROUND OF THE INVENTION

Aluminum beverage containers are generally made in two pieces, one piece forming the container sidewalls and bottom (referred to herein as a "container body") and a second piece forming the container top. Container bodies are formed by methods well known in the art. Generally, the container body is fabricated by forming a cup from a circular blank of aluminum sheet and then extending and thinning the sidewalls by passing the cup through a series of dies having progressively smaller bore size. This process is referred to as "drawing and ironing" the container body.

A common aluminum alloy used to produce container bodies is AA3004, an alloy registered with the Aluminum Association. The physical characteristics of AA 3004 are appropriate for drawing and ironing container bodies due primarily to the relatively low magnesium (Mg) and manganese (Mn) content of the alloy. A desirable characteristic of AA3004 is that the amount of work hardening imparted to the aluminum sheet during the can making process is relatively minor.

Aluminum alloy sheet is most commonly produced by an ingot casting process. In this process, the aluminum alloy material is initially cast into an ingot, for example having a thickness of from about 20 to 30 inches. The ingot is then homogenized by heating to an elevated temperature, which is typically 1075° F. to 1150° F., for an extended period of time, such as from about 6 to 24 hours. The homogenized ingot is then hot rolled in a series of passes to reduce the thickness of the ingot. The hot rolled sheet is then cold rolled to the desired final gauge.

Despite the widespread use of ingot casting, there are numerous advantages to producing aluminum alloy sheet by continuously casting molten metal. In a continuous casting process, molten metal is continuously cast directly into a relatively long thin slab and the cast slab is then hot rolled and cold rolled to produce a finished product. However, not all alloys can be readily cast using a continuous casting process into aluminum sheet that is suitable for forming operations, such as for making drawn and ironed container bodies.

Attempts have been made to continuously cast AA 3004 alloy. For example, in a paper entitled "Production of Continuous Cast Can Body Stock," which was presented by McAuliffe, an employee of the assignee of the present application, on Feb. 27, 1989, at the AIME meeting in Las Vegas, it is disclosed that limited testing was conducted with two manufacturers of 12 ounce, 90 pound cans (i.e., a minimum buckle strength of 90 p.s.i.). One test produced 3004 can stock. The paper discloses that "[b]oth tests, in the 2-3% earring range, verified that the surface and internal quality and structure were sufficient to produce cans of acceptable quality." However, it has been found that the continuously cast AA3004 alloy is unsuitable for typical high carbonation beverages, such as soda, because it has insufficient buckle strength when employed using current

typical stock gauges (e.g., from about 0.0112" to 0.0118") as opposed to stock gauges used at the time of the McAuliffe article (e.g., from about 0.0124" to 0.0128"). This is due to the poor after-bake characteristics of continuously cast AA 3004 alloy that is produced having suitable eating levels. This is discussed in more detail hereinafter in connection with examples of the physical characteristics of continuously cast AA 3004 alloy.

U.S. Pat. No. 4,238,248 by Gyongos et al. discloses casting an AA 3004 type alloy in a block casting apparatus. The alloy had a magnesium content from 0.8 to 1.3 percent and a manganese content from 1.0 to 1.5 percent, with up to 0.25 percent copper. As used throughout the present specification, all percentages refer to weight percent unless otherwise indicated. However, there is no disclosure of processing the cast strip into sheet suitable for container bodies.

U.S. Pat. No. 4,235,646 by Neufeld et al. describes the continuous casting of an AA5017 aluminum alloy that is useful for beverage container bodies and container ends. The alloy includes 0.4 to 1.0 percent manganese, 1.3 to 2.5 percent magnesium and 0.05 to 0.4 percent copper. However, it is also disclosed that "copper and iron are included in the present composition due to their inevitable presence in consumer scrap. The presence of copper between 0.05 and 0.2 percent also enhances the low earring properties and adds to the strength of the present alloy." In Examples 1-3, the copper content of the alloys was 0.04 percent and 0.09 percent. In addition, the process includes a flash anneal step. In one example, the sheet stock disclosed by Neufeld et al. had a yield strength after cold rolling of 278 MPa (40.3 ksi) and an earring percentage of 1.2 percent.

U.S. Pat. No. 4,976,790 by McAuliffe et al. discloses a process for casting aluminum alloys using a block-type strip caster. The process includes the steps of continuously casting an aluminum alloy strip and thereafter introducing the strip into a hot mill at a temperature of from about 880° F. to 1000° F. (471° C.-538° C.). The strip is hot rolled to reduce the thickness by at least 70 percent and the strip exits the hot roll at a temperature of no greater than 650° F. (343° C.). The strip is then coiled to anneal at 600° F. to 800° F. (316° C.-427° C.) and is then cold rolled, annealed and subjected to further cold rolling to optimize the balance between the 45° earring and the yield strength. The preferred annealing temperature after cold rolling is 695° F. to 705° F. (368° C.-374° C.).

U.S. Pat. No. 4,517,034 by Merchant et al. describes a method for continuously casting a modified AA 3004 alloy composition which includes 0.1 to 0.4 percent chromium. The sheet stock has an eating percentage of 3.12 percent or higher.

U.S. Pat. No. 4,526,625 by Merchant et al. also describes a method for continuously casting an AA 3004 alloy composition which is alleged to be suitable for drawn and ironed container bodies. The process includes the steps of continuously casting an alloy, homogenizing the cast alloy sheet at 950° F.-1150° F. (510° C.-621° C.), cold rolling the sheet, and annealing the sheet at 350° F.-550° F. (177° C.-288° C.) for a time of about 2-6 hours. The sheet is then cold rolled and reheated to recrystallize the grain structure at 600° F.-900° F. (316° C.-482° C.) for about 1-4 hours. The sheet is then cold rolled to final gauge. The reported earring for the sheet is about 3 percent or higher.

U.S. Pat. No. 5,192,378 by Doherty et al. discloses a process for making an aluminum alloy sheet useful for forming into container bodies. The aluminum alloy includes

1.1–1.7 percent magnesium, 0.5–1.2 percent manganese and 0.3–0.6 percent copper. The cast ingot is homogenized at 900° F.–1080° F. for about 4 hours, hot rolled, annealed at 500° F.–700° F., cold rolled and then annealed at 750°–1050° F. The body stock can have a yield strength of 40–52 ksi after the final cold rolling.

U.S. Pat. No. 4,111,721 by Hitchler et al. discloses a process for continuously casting AA 3004 type alloys. The cast sheet is held at a temperature of at least about 900° F. (482° C.) for from about 4 to 24 hours prior to final cold reduction.

European Patent Application No. 93304426.5 discloses a method and apparatus for continuously casting aluminum alloy sheet. It is disclosed that an aluminum alloy having 0.93 percent manganese, 1.09 percent magnesium and 0.42 percent copper and 0.48 percent iron was cast into a strip. The composition was hot rolled in two passes and then solution heat treated continuously for 3 seconds at 1000° F. (538° C.), quenched and cold rolled to final gauge. Can bodies made from the sheet had an caring of 2.8 percent, a tensile yield strength of 43.6 ksi (301 MPa). An important aspect of the invention disclosed in European Patent Application No. 93304426.5 is that the continuously cast strip be subjected to solution heat treating immediately after hot rolling without intermediate cooling, followed by a rapid quench. In fact, it is illustrated in Example 4 that strength is lost when the solution heat treatment and quenching steps of the invention are replaced with a conventional batch coil annealing cycle and cold working is limited to about 50 percent to maintain required eating, as is typical in continuous cast processes. Solution heat treating is disadvantageous because of the high capital cost of the necessary equipment and the increased energy requirements.

There remains a need for a process which produces an aluminum alloy sheet having sufficient strength and formability characteristics to be easily made into drawn and ironed beverage containers. The sheet stock should have good strength and elongation, and the resulting container bodies should have low caring.

It would be desirable to have a continuous aluminum casting process in which there is no need for a heat soak homogenization step. It would be advantageous to have a continuously cast process in which it is unnecessary to continuously anneal and solution heat treat the cast strip immediately following hot rolling (e.g., without intermediate cooling) followed by immediate quenching. It would be advantageous to have an aluminum alloy suitable for continuous casting in which the grain size is sufficient to provide for enhanced formability. It would be desirable to have an aluminum alloy suitable for continuous casting in which the magnesium level is kept low in order to achieve comparable brightness when compared to commercially available continuous cast can stock. It would be desirable to have an aluminum alloy suitable for continuous casting which can be formed into containers having suitable formability and having low caring and suitable strength.

#### SUMMARY OF THE INVENTION

In accordance with the present invention, a method is provided for fabricating an aluminum sheet product. The method includes the following steps. An aluminum alloy melt is formed which includes from about 0.7 to about 1.3 weight percent manganese, from about 1.0 to about 1.5 weight percent magnesium, from about 0.3 to about 0.6 weight percent copper, up to about 0.5 weight percent silicon, and from about 0.3 to about 0.7 weight percent iron,

the balance being aluminum and incidental additional materials and impurities. In a preferred embodiment, the aluminum alloy melt includes from about 1.15 to about 1.45 weight percent magnesium and more preferably from about 1.2 to about 1.4 weight percent magnesium, from about 0.75 to about 1.2 weight percent manganese and more preferably from about 0.8 to about 1.1 weight percent manganese, from about 0.35 to about 0.5 weight percent copper and more preferably from about 0.38 to about 0.45 weight percent copper, from about 0.4 to about 0.65 weight percent iron and more preferably from about 0.50 to about 0.60 weight percent iron, and from about 0.13 to about 0.25 weight percent silicon, with the balance being aluminum and incidental additional materials and impurities. The alloy melt is continuously cast to form a cast strip and the cast strip is hot rolled to reduce the thickness and form a hot rolled strip. The hot rolled strip can be subsequently cold rolled without any intervening hot mill anneal step or can be annealed after hot rolling for at least about 0.5 hours at a temperature from about 700° F. to about 900° F. to form a hot mill annealed strip. The hot rolled strip or hot mill annealed strip is cold rolled to form a cold rolled strip wherein the thickness of the strip is reduced to the desired intermediate anneal gauge, preferably by about 35% to about 60% per pass. The cold rolled strip is annealed to form an intermediate cold mill annealed strip. The intermediate cold mill annealed strip is subjected to further cold rolling to reduce the thickness of the strip and form aluminum alloy strip stock.

In accordance with the present invention, aluminum alloy strip stock is provided comprising from about 0.7 to about 1.3 weight percent manganese, from about 1.0 to about 1.5 weight percent magnesium, from about 0.38 to about 0.45 weight percent copper, from about 0.50 to about 0.60 weight percent iron and up to about 0.5 weight silicon, with the balance being aluminum and incidental additional materials and impurities. The aluminum alloy strip stock is preferably made by continuous casting. Preferably, the strip stock has a final gauge after-bake yield strength of at least about 37 ksi, more preferably at least about 38 ksi and more preferably at least about 40 ksi. The strip stock preferably has an eating of less than 2 percent and more preferably less than 1.8 percent.

In accordance with the present invention, a continuous process for producing aluminum sheet is provided. In accordance with the process, relatively high reductions in gauge can be achieved in both the hot mill and cold mill. Additionally, due to the fact that greater hot mill and cold mill reductions are possible, the number of hot roll and cold roll passes can be reduced as compared to commercially available continuously cast can body stock. A relatively high proportion of cold work is needed to produce can body stock having acceptable physical properties according to the sheet production process of the present invention, as compared to commercially available continuously cast can body stock. Thus, a reduced amount of work hardening is imparted to the sheet when it is manufactured into items such as drawn and ironed containers, when compared to commercially available continuously cast can body stock.

In accordance with the present invention, the need for a high temperature soak (i.e., homogenization) can be avoided. When the high temperature homogenization step is performed when the metal is coiled, it can result in pressure welding such that it is impossible to unroll the coil. Also, the need for solution heat treatment after the hot mill (e.g., as disclosed in European Patent Application No. 93304426.5) can be avoided. By avoiding solution heat treatment, the continuous casting process is more economical and results in fewer process control problems.

In accordance with the present process, high amounts of recycled aluminum can be advantageously employed. For example, 75 percent and preferably up to 95 percent or more of used beverage containers (UBC) can be employed to produce the continuous cast sheet of the present invention. The use of increased amounts of UBC significantly reduces the cost associated with producing the aluminum sheet.

In accordance with the present invention, a continuous cast alloy is provided which includes relatively high levels of copper (e.g., 0.3 to 0.6 percent). It has surprisingly been found that the copper can be increased to these levels without negatively affecting the eating. If copper is increased in ingot cast processes, the resulting alloy can be too strong for can-making applications. In addition, in accordance with the present invention, relatively low levels of magnesium are used (e.g., 1.0 to 1.5 percent), leading to better can surface finish than commercially available continuously cast can body stock. For example, when drawn and ironed cans manufactured from aluminum sheet according to the present invention are subjected to industrial washing, less surface etching takes place and, therefore, a brighter can results. Also, the relatively low magnesium content decreases the work hardening rate. Also in accordance with the present invention, a relatively high iron content compared to commercially available continuous cast can body stock is employed to increase formability. It is believed that formability is increased because the increased iron changes the microstructure resulting in a finer grain material, when compared to a low iron content continuously cast material. The tolerance of these high iron levels also increases the amount of UBC that can be utilized, since iron is a common contaminant in consumer scrap.

#### BRIEF DESCRIPTION OF THE DRAWING

The FIGURE is a block diagram illustrating one embodiment of the process of the present invention.

#### DETAILED DESCRIPTION

In accordance with the present invention, aluminum sheet having good strength and forming properties is provided. In addition, a process for producing aluminum sheet is also provided. The resulting aluminum sheet is particularly suitable for the fabrication of drawn and ironed articles, such as containers. The resulting sheet has reduced earing and improved strength in thinner gauges than comparable sheet fabricated according to the prior art.

The preferred aluminum alloy composition according to the present invention includes the following constituents: (1) manganese, preferably with a minimum of at least about 0.7 percent manganese and more preferably with a minimum of at least about 0.75 percent manganese and more preferably with a minimum of at least about 0.8 percent manganese, and preferably with a maximum of at most about 1.3 percent manganese and more preferably with a maximum of at most about 1.2 percent manganese and more preferably with a maximum of at most about 1.1 percent manganese; (2) magnesium, preferably with a minimum of at least about 1.0 percent magnesium and more preferably with a minimum of at least about 1.15 percent magnesium and more preferably with a minimum of at least about 1.2 percent magnesium, and preferably with a maximum of at most about 1.5 percent magnesium and more preferably with a maximum of at most about 1.45 percent magnesium and more preferably with a maximum of at most about 1.4 percent magnesium; (3) copper, preferably with a minimum of at least about 0.3 percent copper and more preferably with a minimum of at

least about 0.35 percent copper and more preferably with a minimum of at least about 0.38 percent copper, and preferably with a maximum of at most about 0.6 percent copper and more preferably with a maximum of at most about 0.5 percent copper and more preferably with a maximum of at most about 0.45 percent copper; (4) iron, preferably with a minimum of at least about 0.3 percent iron and more preferably with a minimum of at least about 0.4 percent iron and more preferably with a minimum of at least about 0.50 percent iron, and preferably with a maximum of at most about 0.7 percent iron and more preferably with a maximum of at most about 0.65 percent iron and more preferably with a maximum of at most about 0.60 percent iron; (5) silicon, preferably with a minimum of 0 percent silicon and more preferably with a minimum of at least about 0.13 percent silicon, and preferably with a maximum of at most about 0.5 percent silicon and more preferably with a maximum of at most about 0.25 percent silicon. The balance of the alloy composition consists essentially of aluminum and incidental additional materials and impurities. The incidental additional materials and impurities are preferably limited to about 0.05 weight percent each, and the sum total of all incidental additional materials and impurities preferably does not exceed about 0.15 percent.

While not wishing to be bound by any theory, it is believed that the copper content of the alloy composition according to the present invention, particularly in combination with the process steps discussed below, contributes to the increased strength of the aluminum alloy sheet stock while maintaining acceptable elongation and earing characteristics. Additionally, it is believed that the relatively low level of magnesium results in a brighter finish in containers manufactured from the alloy of the present invention, due to a decrease in surface etching, when compared to currently commercially available continuously cast stock. Furthermore, it is believed that the relatively high level of iron leads to increased formability because the iron changes the microstructure resulting in a finer grain material when compared to continuous cast materials cast with similar levels of manganese, copper and magnesium and, having lower levels of iron.

According to a preferred embodiment of the present invention, a continuous casting process is used to form an aluminum alloy melt into an aluminum alloy sheet product. The continuous casting process can employ a variety of continuous casters, such as a belt caster or a roll caster. Preferably, the continuous casting process includes the use of a block caster for casting the aluminum alloy melt into a sheet. The block caster is preferably of the type disclosed in U.S. Pat. Nos. 3,709,281; 3,744,545; 3,747,666; 3,759,313 and 3,774,670 all of which are incorporated herein by reference in their entirety.

According to this embodiment of the present invention, a melt of the aluminum alloy composition described above is formed. The alloy composition according to the present invention can be formed in part from scrap material such as plant scrap, can scrap and consumer scrap. Plant scrap can include ingot scalings, rolled strip slicings and other alloy trim produced in the mill operation. Can scrap can include scrap produced as a result of earing and galling during can manufacture. Consumer scrap can include containers recycled by users of beverage containers. It is preferred to maximize the amount of scrap used to form the alloy melt and preferably the alloy composition according to the present invention is formed with at least about 75 percent and preferably at least about 95 percent total scrap.

In order to come within the preferred elemental ranges of the present alloy, it is necessary to adjust the melt. This may

be carried out by adding elemental metal, such as magnesium or manganese, or by adding unalloyed aluminum to the melt composition to dilute excess alloying elements.

The metal is charged into a furnace and is heated to a temperature of about 1385° F. to thoroughly melt the metal. The alloy is treated to remove materials such as dissolved hydrogen and non-metallic inclusions which would impair casting of the alloy and the quality of the finished sheet. The alloy can also be filtered to further remove non-metallic inclusions from the melt.

The melt is then cast through a nozzle and into the casting cavity. The nozzle is typically fabricated from a refractory material and provides a passage from the melt to the caster wherein the molten metal is constrained by a long narrow tip upon exiting the nozzle. For example, a nozzle tip having a thickness of from about 10 to about 25 millimeters and a width of from about 254 millimeters to about 2160 millimeters can be used. The melt exits the tip and is received in a casting cavity formed by opposite pairs of rotating chill blocks.

The metal cools as it travels within the casting cavity and solidifies by transferring heat to the chill blocks until the strip exits the casting cavity. At the end of the casting cavity, the chill blocks separate from the cast strip and travel to a cooler where the chill blocks are cooled. The rate of cooling as the cast strip passes through the casting cavity of the casting apparatus is a function of various process and product parameters. These parameters include the composition of the material being cast, the strip gauge, the chill block material, the length of the casting cavity, the casting speed and the efficiency of the block cooling system.

It is preferred that the cast strip exiting the block caster be as thin as possible to minimize subsequent working of the strip. Normally, a limiting factor in obtaining minimum strip thickness is the thickness and width of the distributor tip of the caster. In the preferred embodiment of the present invention, the strip is cast at a thickness of from about 12.5 millimeters to about 25.4 millimeters and more preferably about 19 millimeters.

Upon exiting the caster, the cast strip is then subjected to hot rolling in a hot mill. A hot mill includes one or more pairs of oppositely rotating rollers having a gap therebetween that reduce the thickness of the strip as it passes through the gap. The cast strip preferably enters the hot mill at a temperature in the range of from about 850° F. to about 1050° F. According to the process of the present invention, the hot mill preferably reduces the thickness of the strip by at least about 70 percent and more preferably by at least about 80 percent. In a preferred embodiment, the hot mill includes 2 pairs of hot rollers and the percentage reduction in the hot mill is maximized. The hot rolled strip preferably exits the hot mill at a temperature in the range from about 500° F. to about 750° F. In accordance with the present invention, it has been found that a relatively high reduction in gauge can take place in each pass of the hot rollers and therefore the number of pairs of hot rollers can be minimized.

The hot rolled strip is optionally annealed to remove any residual cold work resulting from the hot mill operation and to reduce the earing. Preferably, the hot rolled strip is annealed in a hot mill anneal step at a temperature of a minimum of at least about 700° F. and more preferably a minimum of at least about 800° F., and preferably with a maximum temperature of at most about 900° F. and more preferably a maximum temperature of at most about 850° F. According to one embodiment, a preferred temperature for

annealing is about 825° F. The entire metal strip should preferably be at the annealing temperature for at least about 0.5 hours, more preferably at least about 1 hour and more preferably at least about 2 hours. The amount of time that the entire metal strip should be at the annealing temperature should preferably be a maximum of at most about 5 hours, more preferably a maximum of at most about 4 hours. In a preferred embodiment, the anneal time is about 3 hours. For example, the strip can be coiled, placed in an annealing furnace, and held at the desired anneal temperature for from about 2 to about 4 hours. This length of time insures that interior portions of the coiled strip reach the desired annealing temperature and are held at that temperature for the preferred period of time. It is to be expressly understood that the annealing times listed above are the times for which the entire metal strip is maintained at the annealing temperatures, and these times do not include the heat-up time to reach the anneal temperature and the cool-down time after the anneal soak. The coiled strip is preferably cooled expeditiously to allow further processing, but is not rapidly quenched to retain a solution heat treated structure.

Alternatively, the hot rolled strip is not subjected to a hot mill anneal step. In this alternative embodiment, the hot rolled strip is allowed to cool and is subsequently subjected to cold rolling without any intermediate thermal treatment. It is to be expressly understood that the hot rolled strip is not subjected to a heat soak homogenization, nor is it subjected to a solution heat treatment followed by a rapid quench. The strip is cooled in the manner that is most convenient.

After the hot mill annealed or hot rolled sheet has cooled to ambient temperature, it is cold rolled in a first cold rolling step to an intermediate gauge. Preferably, cold rolling to intermediate gauge includes the step of passing the sheet between one or more pairs of rotating cold rollers (preferably 1 to 3 pairs of cold rollers) to reduce the thickness of the strip by from about 35 percent to about 60 percent per pass through each pair of rollers, more preferably by from about 45 percent to about 55 percent per pass. The total reduction in thickness is preferably from about 45 to about 85 percent. In accordance with the process of the present invention, it has been found that a relatively large reduction in the gauge of the aluminum sheet can take place in each pass as compared to a commercially available continuously cast can stock. In this manner, it is possible to reduce the number of passes required in the cold mill.

When the desired intermediate anneal gauge is reached following the first cold rolling step, the sheet is intermediate cold mill annealed to reduce the residual cold work and lower the earing. Preferably, the sheet is intermediate cold mill annealed at a minimum temperature of at least about 600° F., more preferably at a minimum temperature of at least about 650° F., and preferably at a maximum temperature of no more than about 900° F. and more preferably at a maximum temperature of no more than about 750° F. According to one embodiment, a preferred annealing temperature is about 705° F. The anneal time is preferably a minimum of at least about 0.5 hours and is more preferably a minimum of at least about 2 hours. According to one embodiment of the present invention, the intermediate cold mill anneal step can include a continuous anneal, preferably at a temperature of from about 800° F. to about 1050° F. and more preferably at a temperature of about 900° F. It has unexpectedly been found that these cold mill annealing temperatures lead to advantageous properties.

After the cold rolled and intermediate cold mill annealed sheet has cooled to ambient temperature, a final cold rolling step is used to impart the final properties to the sheet. The

preferred final cold work percentage is that point at which a balance between the ultimate tensile strength and the eating is obtained. This point can be determined for a particular alloy composition by plotting the ultimate tensile strength and earing values against the cold work percentage. Once this preferred cold work percentage is determined for the final cold rolling step, the gauge of the sheet during the intermediate annealing stage and, consequently, the cold work percentage for the first cold roll step can be determined and the hot mill gauge can be optimized to minimize the number of passes.

In a preferred embodiment the reduction to final gauge is from about 45 to about 80 percent, preferably in one or two passes of from about 25 to about 65 percent per pass, and more preferably a single pass of 60 percent reduction. When the sheet is fabricated for drawn and ironed container bodies, the final gauge can be, for example, from about 0.0096 inches to about 0.015 inches.

An important aspect of the present invention is that the aluminum sheet product that is produced in accordance with the present invention can maintain sufficient strength and formability properties while having a relatively thin gauge. This is important when the aluminum sheet product is utilized in making drawn and ironed containers. The trend in the can-making industry is to use thinner aluminum sheet stock for the production of drawn and ironed containers, thereby producing a container containing less aluminum and having a reduced cost. However, to use thinner gauge aluminum sheet stock the aluminum sheet stock must still have the required physical characteristics, as described in more detail below. Surprisingly, a continuous casting process has been discovered which, when utilized with the alloys of the present invention, produces an aluminum sheet stock that meets the industry standards.

The aluminum alloy sheet produced according to the preferred embodiment of the present invention is useful in a number of applications including, but not limited to, drawn and ironed container bodies. When the aluminum alloy sheet is to be fabricated into drawn and ironed container bodies, the alloy sheet preferably has an after-bake yield strength of at least about 37 ksi, more preferably at least about 38 ksi,

10  
15

about 43 ksi. The as rolled ultimate tensile strength is

preferably at least 41 ksi and more preferably at least 42 ksi

and more preferably at least 43 ksi, and preferably, not

greater than 46 ksi and more preferably not greater than 45

ksi and more preferably not greater than 44.5 ksi.

To produce acceptable drawn and ironed container bodies, aluminum alloy sheet should have a low earing percentage. A typical measurement for earing is the 45° earing or 45° rolling texture. Forty-five degrees refers to the position on the aluminum sheet which is 45° relative to the rolling direction. The value for the 45° earing is determined by measuring the height of the ears which stick up in a cup, minus the height of valleys between the ears. The difference is divided by the height of the valleys times 100 to convert to a percentage.

20  
25  
30  
35

Preferably, the aluminum alloy sheet, according to the present invention, has a tested earing of less than about 2 percent and more preferably less than about 1.8 percent. Importantly, the aluminum alloy sheet product produced in accordance with the present invention should be capable of producing commercially acceptable drawn and ironed containers. Therefore, when the aluminum alloy sheet product is converted into container bodies, the eating should be such that the bodies can be conveyed on the conveying equipment and the eating should not be so great as to prevent acceptable handling and trimming of the container bodies.

In addition, the aluminum sheet should have an elongation of at least about 2 percent and more preferably at least about 3 percent and more preferably at least about 4 percent. Further, container bodies fabricated from the alloy of the present invention having a minimum dome reversal strength of at least about 88 psi and more preferably at least about 90 psi at current commercial thickness.

40  
45

## EXAMPLES

In order to illustrate the advantages of the present invention, a number of aluminum alloys were formed into sheets.

Four examples comparing AA 3004/3104 alloys with the alloys of the present invention are illustrated in Table I.

TABLE I

| Example         | Composition (weight %) |      |      |      | Hot mill Anneal | Cold mill Anneal | Secondary |
|-----------------|------------------------|------|------|------|-----------------|------------------|-----------|
|                 | Mg                     | Mn   | Cu   | Fe   | Temperature     | Temperature      | Cold Work |
| 1 (comparative) | 1.21                   | 0.84 | 0.22 | 0.44 | 825° F.         | 705° F.          | 75%       |
| 2 (comparative) | 1.28                   | 0.96 | 0.21 | 0.41 | 825° F.         | 705° F.          | 75%       |
| 3               | 1.22                   | 0.83 | 0.42 | 0.35 | 825° F.         | 705° F.          | 64%       |
| 4               | 1.31                   | 0.99 | 0.41 | 0.34 | 825° F.         | 705° F.          | 61%       |

55  
60  
65

and more preferably at least about 40 ksi. After-bake yield strength refers to the yield strength of the aluminum sheet after being subjected to a temperature of about 400° F. for about 10 minutes. This treatment simulates conditions experienced by a container body during post-formation processing, such as the washing and drying of containers, and drying of films or paints applied to the container. Preferably, the as rolled yield strength is at least 38 ksi and more preferably at least 39 ksi, and preferably is not greater than about 44 ksi and more preferably is not greater than about 43 ksi. The aluminum sheet preferably has an after-bake ultimate tensile strength of at least about 40 ksi, more preferably at least about 41.5 ksi and more preferably at least

and 0.22 and the balance of the composition was aluminum. Each alloy was continuously cast in a block caster and was then continuously hot rolled. The hot mill and intermediate cold mill anneals were each for about 3 hours. After the hot mill anneal, the sheets were cold rolled to reduce the thickness by from about 45 to 70 percent in one or more passes. After this cold rolling, the sheets were intermediate cold mill annealed at the temperature indicated.

Thereafter, the sheets were cold rolled to reduce the thickness by the indicated percentage. Table II illustrates the results of testing the processed sheets.

TABLE II

| Example         | As-Rolled |      |         | After-Bake |      |      |         |
|-----------------|-----------|------|---------|------------|------|------|---------|
|                 | UTS       | YS   | Elonga- | Earing     | UTS  | YS   | Elonga- |
| 1 (comparative) | 41.3      | 39.3 | 3.2%    | 2.2%       | 40.0 | 35.2 | 4.8%    |
| 2 (comparative) | 43.2      | 40.4 | 3.1%    | 2.2%       | 40.7 | 36.0 | 4.3%    |
| 3               | 42.4      | 39.4 | 3.2%    | 1.4%       | 42.3 | 37.1 | 5.1%    |
| 4               | 43.1      | 40.1 | 3.2%    | 1.2%       | 43.3 | 37.8 | 5.3%    |

The ultimate tensile strength (UTS), yield strength (YS), elongation, and earring were each measured when the sheet was in the as-rolled condition. The UTS, YS and elongation were then measured after a bake treatment which consisted of heating the alloy sheet to about 400° F. for about 10 minutes.

Comparative Examples 1 and 2 illustrate that, when fabricated using a continuous caster, an AA 3004/3104 alloy composition is too weak for can-making applications. In order to achieve similar as-rolled strengths, the 3004/3104 alloy requires more cold work, and therefore, has higher earring. Further, the 3004/3104 alloy has a large drop in yield strength after the bake treatment, which can result in a low dome reversal strength for the containers.

Examples 3 and 4 illustrate alloy compositions according to the present invention. The sheets had a significantly lower drop in yield strength due to baking and therefore maintained adequate strength for can-making applications. Further, these alloy sheets maintained low earring. These examples substantiate that AA3004/3104 alloys that are processed in a continuous caster are too weak for use as containers, particularly for carbonated beverages. However, when the copper level is increased according to the present invention, the sheet has sufficient strength for forming cans.

To further illustrate the advantages of the present invention, a number of examples were prepared to demonstrate the effect of increased thermal treatment temperature, such as at temperatures taught by the prior art. These examples are illustrated in Table III.

TABLE III

| Example | Composition |      |      |      | Hot mill            |                                  |
|---------|-------------|------|------|------|---------------------|----------------------------------|
|         | Mg          | Mn   | Cu   | Fe   | Anneal              | Result                           |
| 5       | 1.28        | 0.98 | 0.42 | 0.35 | 1000° F.<br>3 hours | Unable to unwrap<br>coils        |
| 6       | 1.28        | 0.98 | 0.42 | 0.35 | 950° F.<br>3 hours  | Unable to unwrap<br>coils        |
| 7       | 1.28        | 0.98 | 0.42 | 0.35 | 925° F.<br>10 hours | Unable to unwrap<br>4 of 5 coils |

As is illustrated in Table III, annealing temperatures at 925° F. or higher resulted in welded coils which were not able to be unwrapped for further processing. As a result, such temperatures are clearly not useful for alloy sheets according to the present invention.

Table IV illustrates the effect of increasing the iron content according to a preferred embodiment of the present invention.

TABLE IV

| Example | Composition (weight %) |      |      |      | Hot mill Anneal | Intermediate Cold mill Anneal |
|---------|------------------------|------|------|------|-----------------|-------------------------------|
|         | Mg                     | Mn   | Cu   | Fe   | Temperature     | Temperature                   |
| 8       | 1.22                   | 0.83 | 0.42 | 0.38 | 825° F.         | 705° F.                       |
| 9       | 1.31                   | 0.94 | 0.42 | 0.36 | 825° F.         | 705° F.                       |
| 10      | 1.37                   | 1.12 | 0.42 | 0.55 | 825° F.         | 705° F.                       |

In each example in addition to the listed elements, the silicon content was between 0.18 and 0.23 and the balance was essentially aluminum. Each alloy was cast in a block caster and was then continuously hot rolled. The hot mill anneal in all cases was for about 3 hours. After the hot mill anneal, the sheets were cold rolled to reduce the thickness by from about 45 to 70 percent in one or more passes. After this cold rolling, the sheets were intermediate cold mill annealed for about 3 hours at the temperatures indicated and then further cold rolled.

Table V illustrates the results of testing the foregoing aluminum alloy sheets.

TABLE V

| Example | UTS<br>(ksi) | YS<br>(ksi) | Elongation<br>% | Earing<br>% | Result                     |
|---------|--------------|-------------|-----------------|-------------|----------------------------|
| 8       | 42.3         | 37.0        | 5.0             | 1.5         | Excellent for 5.5 oz. cans |
| 9       | 43.2         | 38.2        | 4.8             | 1.6         | Made 12 oz. cans           |
| 10      | 43.2         | 37.8        | 5.2             | 1.7         | Excellent for 12 oz. cans  |

The ultimate tensile strength (UTS), yield strength (YS) and elongation were measured after a bake treatment which consisted of heating the alloy to about 400° F. for about 10 minutes.

Example 8 illustrates an alloy and process according to the present invention for making a sheet product which is sufficient for 5.5 ounce can bodies. By increasing the copper content and maintaining an adequate cold mill anneal temperature, sheet is produced that is excellent for the commercial production of 5.5 ounce container bodies. However, the sheet did not have sufficient formability for the commercial production of 12 ounce container bodies. Although the sheet had sufficient strength and 12 ounce container bodies were made, a commercially unacceptable number of the 12 ounce container bodies were rejected when produced on two commercial can-lines.

Example 9 is similar to Example 8, with increased magnesium and manganese; the sheet was also useful for 5.5 ounce container bodies and did produce some 12 ounce container bodies with acceptable strength. However, the 12 ounce container bodies also had a commercially unacceptable number of rejects.

Example 10 illustrates that by increasing the iron content according to the present invention, this problem can be overcome. In Example 10, the sheet material had excellent fine grain size and was used to produce 12 ounce container bodies on two commercial container lines with a commercially acceptable rate of rejection.

In an alternative embodiment of the present invention, fine grain size may be imparted to the sheet material by using a continuous intermediate cold mill anneal. In one example, an aluminum alloy sheet having the composition illustrated for Example 4 was intermediate cold mill annealed in a continuous, gas-fired furnace wherein the

metal was exposed to a peak temperature of about 900° F. This treatment imparted a very fine grain size to the sheet. The sheet had an ultimate tensile strength of 45.5 ksi and 12 ounce container bodies were produced that met commercial strength requirements.

While various embodiments of the present invention have been described in detail, it is apparent that modifications and adaptations of those embodiments will occur to those skilled in the art. It is to be expressly understood that such modifications and adaptations are within the spirit and scope of the present invention.

What is claimed is:

1. A method for fabricating an aluminum sheet product, comprising the steps of:

- (a) forming an aluminum alloy melt comprising;
  - (i) from about 0.7 to about 1.3 weight percent manganese,
  - (ii) from about 1.0 to about 1.5 weight percent magnesium,
  - (iii) from about 0.3 to about 0.6 weight percent copper,
  - (iv) up to about 0.5 weight percent silicon, and
  - (v) from about 0.3 to about 0.7 weight percent iron, the balance being aluminum and incidental additional materials and impurities;
- (b) continuously casting said alloy melt to form a cast strip;
- (c) hot rolling said cast strip to reduce the thickness of said cast strip and form a hot rolled strip;
- (d) cold rolling said hot rolled strip to form a cold rolled strip wherein the thickness of said hot rolled strip is reduced by from about 35 percent to about 60 percent per pass;
- (e) annealing said cold rolled strip to form an intermediate cold mill annealed strip; and
- (f) further cold rolling said intermediate cold mill annealed strip to reduce the thickness of the strip and form aluminum alloy strip stock;

wherein said aluminum alloy strip stock has an after-bake yield strength of at least about 37 ksi and an earring of less than about 2 percent.

2. A method as recited in claim 1, wherein said aluminum alloy melt comprises from about 0.35 to about 0.5 weight percent copper.

3. A method as recited in claim 1, wherein said hot rolling step reduces the gauge of said cast strip by at least about 70 percent.

4. A method as recited in claim 1, wherein said method comprises the step of either:

- (i) annealing said hot rolled strip for at least about 0.5 hour at a temperature of from about 700° F. to about 900° F. to form a hot mill annealed strip; or
- (ii) cooling said hot rolled strip; immediately after said hot rolling step.

5. A method as recited in claim 1, further comprising the step of annealing said hot rolled strip immediately after said hot rolling step for at least about 0.5 hour at a temperature of from about 700° F. to about 900° F.

6. A method as recited in claim 5, wherein said step of annealing said hot rolled strip comprises heating said hot rolled strip at a temperature of from about 800° F. to about 850° F.

7. A method as recited in claim 6, wherein said step of annealing said cold rolled strip comprises annealing said cold rolled strip for about 3 hours.

8. A method as recited in claim 5, wherein the cooling of said strip from said hot mill annealing step is for at least about 0.5 hour.

9. A method as recited in claim 1, wherein said step of annealing said hot rolled strip comprises annealing said hot rolled strip for from about 1 to about 5 hours.

10. A method as recited in claim 1, wherein said step of annealing said cold rolled strip comprises annealing said cold rolled strip at a temperature of from about 600° F. to about 900° F. in a batch anneal oven.

11. A method as recited in claim 1, wherein said aluminum alloy strip stock has an elongation of at least about 2 percent.

12. A method as recited in claim 1, wherein said step of further cold rolling said cold mill annealed strip comprises cold rolling said cold mill annealed strip to reduce the thickness of said cold mill annealed strip by from about 45 percent to about 80 percent.

13. A method as recited in claim 1, wherein said step of hot rolling said cast strip occurs sequentially after said step of continuously casting without any intermediate heat treatment step.

14. A method as recited in claim 1, wherein said aluminum alloy melt comprises at least about 75 weight percent scrap.

15. A method as recited in claim 1, wherein said aluminum alloy melt comprises at least about 95 weight percent scrap.

16. A method as recited in claim 1, wherein said iron level is selected such that the resultant microstructure, in said strip stock is a fine grain microstructure.

17. A method as recited in claim 1, further comprising the step of forming said aluminum strip stock into drawn and ironed containers.

18. A method as recited in claim 1, wherein the annealing of said cold rolled strip is at a temperature of from about 800° F. to about 1050° F. in a continuous anneal step.

19. An aluminum sheet product produced by the method of claim 1.

20. A method for fabricating an aluminum alloy strip stock, comprising the steps of:

- (a) forming an aluminum alloy melt derived from at least about 75 weight percent scrap, comprising;
  - (i) from about 0.7 to about 1.3 weight percent manganese;
  - (ii) from about 1.0 to about 1.5 weight percent magnesium;
  - (iii) from about 0.35 to about 0.5 weight percent copper;
  - (iv) up to about 0.5 weight percent silicon; and
  - (v) from about 0.4 to about 0.65 weight percent iron, the balance being aluminum and incidental additional materials and impurities;
- (b) continuously casting said alloy melt to form a cast strip;
- (c) hot rolling said cast strip to reduce the thickness of said cast strip by at least about 70 percent to form a hot rolled strip;
- (d) annealing said hot rolled strip for at least about 0.5 hour at a temperature of from about 700° F. to about 900° F. to form a hot mill annealed strip;
- (e) cooling said hot mill annealed strip for at least about 0.5 hour;
- (f) cold rolling said hot mill annealed strip to form a cold rolled strip wherein the thickness of said hot mill annealed strip is reduced by from about 35% to about 60% per pass;
- (g) annealing said cold rolled strip to form a cold mill annealed strip by either:
  - (i) batch annealing at a temperature of from about 650° F. to about 750° F.; or;

- (ii) continuous annealing at a temperature of from about 800° F. to about 1050° F.; and
  - (h) further cold rolling said cold mill annealed strip to reduce the thickness of the strip and form aluminum alloy strip stock;
- wherein said aluminum alloy strip stock has an after-bake yield strength of at least about 37 ksi and an earing of less than about 2 percent.

21. An aluminum alloy strip stock produced by the process of claim 20.

22. Aluminum alloy strip stock produced by continuous casting, comprising:

- (a) from about 0.7 to about 1.3 weight percent manganese;
- (b) from about 1.0 to about 1.5 weight percent magnesium;
- (c) from about 0.38 to about 0.45 weight percent copper;
- (d) from about 0.50 to about 0.60 weight percent iron;
- (e) up to about 0.5 weight percent silicon, the balance being aluminum and incidental additional materials and impurities;

wherein said strip stock has an after-bake yield strength of at least about 37 ksi and earing of less than about 2 percent.

23. The aluminum alloy strip stock as claimed in claim 22, comprising from about 0.75 to about 1.2 weight percent manganese.

24. The aluminum alloy strip stock of claim 22, comprising from about 0.80 to about 1.1 weight percent manganese.

25. The aluminum alloy strip stock of claim 22, comprising from about 1.15 to about 1.45 weight percent magnesium.

26. The aluminum alloy strip stock of claim 22, comprising from about 1.2 to about 1.4 weight percent magnesium.

27. The aluminum alloy strip stock of claim 22, comprising from about 0.13 to about 0.25 weight percent silicon.

28. The aluminum alloy strip stock of claim 22, wherein said strip stock has an after-bake yield strength of at least 38 ksi.

29. The aluminum alloy strip stock of claim 22, wherein said strip stock has an after-bake yield strength of at least 40 ksi.

30. The aluminum alloy strip stock of claim 22, wherein said strip stock has an after-bake ultimate tensile strength of at least 40 ksi.

31. The aluminum alloy strip stock of claim 22, wherein said strip stock has an after-bake ultimate tensile strength of at least 41.5 ksi.

32. The aluminum alloy strip stock of claim 22, wherein said strip stock has an after-bake ultimate tensile strength of at least 43 ksi.

33. The aluminum alloy strip stock of claim 22, wherein said strip stock has earing of less than 1.8 percent.

34. The aluminum alloy strip stock of claim 22, wherein said strip stock has an elongation of greater than 2.0 percent.

35. The aluminum alloy strip stock of claim 22, wherein said strip stock has an elongation of greater than 3.0 percent.

36. The aluminum alloy strip stock of claim 22, wherein said strip stock has an elongation of greater than 4.0 percent.

37. The aluminum alloy strip stock of claim 22, wherein said strip stock is capable of being made into a drawn and ironed container having an average dome thickness of from about 0.0096 inches to about 0.015 inches and a minimum dome reversal strength of about 90 psi.

38. An aluminum alloy sheet produced by a method comprising the steps of:

- (a) forming an aluminum alloy melt comprising:
    - (i) from about 0.7 to about 1.3 weight percent manganese,
    - (ii) from about 1.0 to about 1.5 weight percent magnesium,
    - (iii) from about 0.3 to about 0.6 weight percent copper,
    - (iv) up to about 0.5 weight percent silicon, and
    - (v) from about 0.3 to about 0.7 weight percent iron, the balance being aluminum and incidental additional materials and impurities;
  - (b) continuously casting said alloy melt to form a cast strip;
  - (c) hot rolling said cast strip to reduce the thickness of said cast strip and form a hot rolled strip;
  - (d) annealing said hot rolled strip for at least about 0.5 hour at a temperature of from about 700° F. to about 900° F. to form a hot mill annealed strip;
  - (e) cold rolling said hot mill annealed strip to form a cold rolled strip wherein the thickness of said hot mill annealed strip is reduced by from about 35 percent to about 60 percent per pass;
  - (f) annealing said cold rolled strip by either:
    - (i) batch annealing at a temperature of from about 600° F. to about 900° F. to form a cold mill annealed strip; or
    - (ii) continuous annealing at a temperature from about 800° F. to about 1050° F. to form a cold mill annealed strip; and
  - (g) further cold rolling said cold mill annealed strip to reduce the thickness of the strip and form aluminum alloy strip stock;
- wherein said aluminum alloy strip stock has an after-bake yield strength of at least about 37 ksi and an earing of less than about 2 percent.

\* \* \* \* \*